

Aug. 29, 1944.

J. S. NACHTMAN

2,357,126

## ALLOYING AND FUSING PROCESS

Filed May 5, 1938

3 Sheets-Sheet 1



John S. Nachtmann

By Holter, Pierce & Scheffler  
Attorneys.

Aug. 29, 1944.

J. S. NACHTMAN

2,357,126

ALLOYING AND FUSING PROCESS

Filed May 5, 1938

3 Sheets-Sheet 2



Fig. 4.



Fig. 3.

John S. Nachtmann

By Potter, Pierce & Scheffler

Attorneys.

Aug. 29, 1944.

J. S. NACHTMAN

2,357,126

ALLOYING AND FUSING PROCESS

Filed May 5, 1938

3 Sheets-Sheet 3



John S. Nachtman

By Potter, Pierce and Scheffler

Attorneys.

## UNITED STATES PATENT OFFICE

2,357,126

## ALLOYING AND FUSING PROCESS

John S. Nachtman, Beaver, Pa.

Application May 5, 1938, Serial No. 206,257

5 Claims. (Cl. 204—28)

The present invention relates to methods and apparatus for applying a finishing treatment—although not necessarily the final treatment—to coated strip metal such as a sheet metal base carrying a film or layer of metal, e. g., electro-deposited metal, on a surface thereof.

The common hot-dip method involving, for example, the application of tin to strip steel, produces a coating generally poor in quality both as to uniformity and appearance. Electrodeposition alone, particularly in continuous high-speed processes, tends to produce a coating which, while having a better appearance and an improved uniformity, has localized areas wherein the strength of union or adherence of coating to base metal is too low. This problem is increased where the union is between the deposited metal and steel of relatively low carbon content.

Accordingly, it is the primary object of the present invention to devise and provide a method of treatment, and apparatus therefor, resulting in the production of a surface coating which is uniform in thickness, smooth and bright in appearance, and firmly and uniformly united to the base metal.

More specifically, this invention contemplates the formation of a sub-surface alloy zone between the base metal and a previously applied surface coating of metal with substantially simultaneous fusing of the surface coating—followed, of course, by cooling the fused material to solidification. In its preferred form the method comprises the steps of preheating the coated strip to a temperature approaching but below the fusing point of the coating; increasing the temperature sufficiently, or subjecting the strip to an already existing higher temperature that is sufficient to produce fusion of the coating; and quick-chilling the strip to cause a rapid solidification of the fused material.

In the first step, some alloy is formed between the base metal and the coating, and the use of a preheating chamber also affords increased efficiency and permits a shortening of the actual fusion chamber associated therewith. A minimum possible shortness of the fusion chamber is desirable where an elongated or continuous strip is conveyed therethrough, as such a strip cannot well be supported (e. g., cannot be physically contacted) while its coating is in a partially molten condition. Most of the total heat required is used to raise the temperature of the base metal, and hence the temperature for preheating is made as high in each case as can be without rendering the coating soft and sticky.

During the carrying out of the fusing step, in the fusion chamber, there is a further alloying of the base metal and its coating, the degree or amount of which is determined by the temperature of the strip and the time period during which the strip is subjected to such temperature. When the coated strip being treated is subjected to the heating zones for only a few seconds the amount of alloy formed is difficult to detect: nevertheless, the coating is brightened and is united to the base metal more firmly than it was prior to the treatment.

In the following cooling step, in the cooling chamber, the temperature of the strip, or at least of the coating, is quickly reduced and held to a value below the solidification point of the coating material, thus stopping the alloying action and simultaneously solidifying or hardening the fused metal into a continuous coating of excellent uniformity and fine appearance.

The heat source or sources for the preheating and fusing steps may be of any suitable character and arrangement. For example, electrical heating elements may be disposed within the preheating and/or fusing chamber. In some instances a liquid or gaseous medium may be heated exteriorly of the chamber or chambers and circulated therethrough. Likewise the chilling means may be varied in form and arrangement.

If the nature of the coating metal is such that a damaging oxidation takes place in the presence of air in any of the chambers, e. g., wherein the strip and/or coating is maintained at elevated temperature, provision will be made for supplying a reducing atmosphere, or non-oxidizing atmosphere, in one or more of the chambers. This can be done in various suitable ways, including simply the injection of reducing gases into such chambers in sufficient volume to displace all or most of the air. In the heating chambers the result is obtainable in desirable manner either by employing, as a heat source, gas jets burning with reducing flame, or by utilizing a heat-transmitting medium such as oil so that use can be made of the reducing vapors or gases given off by the hot medium.

The major objects of the present invention will be apparent from the preceding discussion. Further important objects reside in the provision of novel and useful apparatus in several forms for effectively treating a strip of coated material in the manner set forth, and other objects will appear as the description proceeds.

The drawings accompanying this specification consist of the following illustrations:

Fig. 1 is a side elevational view, with portions of the supporting structure in section, of a preferred form of apparatus constituting a part of this invention;

Fig. 2 represents a vertical section taken substantially on the plane of line 2—2, Fig. 1, looking in the direction of the arrows;

Fig. 3 represents a further vertical section taken on a plane normal to that of Fig. 2, substantially on the plane of line 3—3 of Fig. 2, looking in the direction of the arrows;

Fig. 4 is a view similar to Fig. 3, but showing a somewhat modified form of apparatus;

Fig. 5 represents, in section on the order of Figs. 3 and 4, a still further modified form of apparatus.

With continued reference to the drawings, wherein like characters are employed to designate like parts, and with particular reference for the moment to Figs. 1 to 3, the numeral 7 designates, let us say, a very long, i. e., "continuous" strip of sheet steel that has passed continuously through a series of treating apparatus and has just come through a plating bath where it received, by electrodeposition, a surface coating of metal, e. g., of tin. It is shown entering into, passing through and emerging from the apparatus of the present invention, indicated generally and in its entirety by the numeral 8.

The apparatus 8 has a shaping and supporting framework including vertical corner stanchions 9 intertiered by cross members 10, the stanchions projecting downwardly into a pit 12 below a floor 13. This framework carries four vertical walls 14, properly joined and sealed at their edges to form a rectangular tank closed at the bottom by a plate 15. The tank is substantially filled with liquid as indicated, and by means of a horizontal baffle plate 16 and a vertical partition 17 the tank is divided into a pair of chambers 18 and 19, hereafter referred to respectively as the fusing and chilling chambers. The partition 17 is a hollow double-walled structure filled with a heat-insulating material 20.

The chambers 18 and 19 open upwardly into a hood 22 and have individual stack vents 23 and 24, separated by the upper part of the partition 17. The vent 23 preferably is provided with a damper 25. Two of the hood walls, as shown (Fig. 3), are inclined to overhang two of the walls 14 and form therewith and with a pair of added vertical walls 26 and 27, a pair of chambers 28 and 29 hereafter referred to respectively as the pre-heating and exit chambers. The walls 26 and 27 are approximately U-shaped in cross section, and the former is covered with heat-insulating material 30.

The bottom of chamber 28 is formed by a platform 31 upon which is mounted a pair of entrance rolls 32 which pinch and feed the strip 7 into said chamber. One of these rolls is driven by a motor 33 (Fig. 2). The strip passes upwardly, centrally of the chamber 28, to a driven guide roll 34, the latter being disposed within hood 22 and having a shaft 35 driven by a motor 36 and mounted in bearings 37. This guide roll is so located that the strip then passes downwardly centrally of the chamber 18 through a slot 38 in the baffle 16 and thence to a second guide roll 39. The latter is journaled in bearings 40 so disposed that the strip can be drawn off toward the center of the upper section of the chamber 19. Atop the chamber 19 and above the liquid level there is disposed a pair of rolls, 42, 43 (Fig. 3) which serves as a squeegee and guide assembly for the 75

traveling strip. The strip preferably is then drawn downwardly toward floor level to leave the apparatus by way of a delivery roll 44 and thence either to be reeled or to be passed on for further treatment. A platform 45 carries the roll 44, and a shielding wall 27 preferably is provided to protect the strip in its passage to said roll.

One of the walls 14 has a removable cover 47 for facilitating assembly, adjustment and repair of some of the parts.

As previously stated, the preheating and fusing may be done in any manner suitable for obtaining the requisite temperatures. The illustrated embodiment of preheating means comprises two banks of electrical heating elements 48 arranged in the chamber 28 on opposite sides of the strip 7 and controlled by a thermostat 49 which is adjusted to afford a chamber temperature that will cause some alloying between the coating metal and the steel without actually fusing the coating metal. If the coating material happens to be such as will oxidize readily, reducing gas may be caused to pass from the hood above the fusion chamber 18 into the chamber 28 by closing the damper 25. In some cases, sufficient preheating temperatures are obtainable by conduction through and radiation from the wall between the fusing and preheating chambers.

The liquid in the fusion chamber 18 may likewise be heated by banks of electrical units, 50, under the control of one or more thermostats 52 that are adjusted to afford a temperature that will cause the coating to fuse and flow sufficiently to spread uniformly and smoothly over the surface of the base metal; at the temperature of the fusion chamber the coating further alloys itself simultaneously with the base metal of the strip. The liquid heat-transmitting medium may consist of oil or oily medium with a sufficiently high flash point and no appreciable tendency to attack the metal coating.

The baffle plate 16 tends to prevent liquid circulation and heat exchange between the chilling and fusion chambers. It minimizes the formation of eddy currents by the moving strip.

Almost immediately after passing the baffle the strip 7 has its coating chilled and hardened by the impingement thereon of jets of cooling liquid which come from opposed sets of immersed pipes 53 designed to spray the cold liquid toward the two surfaces of the strip. These pipes connect to manifolds or headers 54 externally of the chamber and the manifolds in turn connect by way of a pipe 55 to the discharge side of a liquid cooling and circulating unit that comprises a pump 56 and a heat exchanger 57 (Fig. 1). The exchanger has the usual connections 58, 59 for circulation therethrough of a separate heat removing liquid.

The intake side of the pump 56 is designed to withdraw the heat-transmitting oil or other liquid from the chilling chamber 19, and, to effectively accomplish this, the withdrawal is effected at three points by means of a pipe 60 having branches 62, 63, the branch 63 in turn having a branch 64. Each branch is equipped with a valve, as shown, for manually regulating the flow through each and thus controlling the chamber temperatures at and adjacent the points where the branches enter the chamber.

The branch 62 enters the bottom of the chilling chamber and is regulated to draw off just enough liquid to ensure constant mixture or internal circulation of the liquid. Branch 63 is connected

to a manifold 65 from which a pair of pipes 66 project into the chamber immediately adjacent the baffle 16. Best temperature conditions are obtained by removing most of the total withdrawn liquid through these pipes 66. The third branch, 64, terminates in a pipe section 67 that is disposed in the extreme upper part of the chilling chamber (Fig. 3). In some instances, where the heat-transmitting or chilling liquid is viscous it will be desirable to use this pipe section, or added heating elements adjacent thereto, to heat the surface portion of the liquid and render it readily removable by the squeegee assembly 42, 43.

As shown in Fig. 2, a chamber 68 containing a float 69 may be provided in communication with the upper part of the liquid body, with the float connected to an electrical switch device 70 for the purpose of maintaining the desired constant liquid level, in obvious manner, with the switch device in circuit with means governing the liquid supply. Obviously, the control for the heating units, 50, may be connected in this circuit so that the heat will be disconnected if liquid level falls too far.

The mode of operation of the above described apparatus and the results obtained thereby in the several successive steps should now be well understood, and a detailed summary therefore is believed unnecessary. The preheating step has several functions as above set forth, but its primary purpose is to bring the entire strip to a temperature approaching but short of the fusion temperature of the coating, thus permitting the fusion chamber to be of a desirably short length. The vertical stretch of the strip is preferable for passage through the fusion chamber as it aids in producing a rapid and uniform spreading of the fused metal, and supports the strip without tendency to distort or to deflect. Hence the slot 38 in the baffle may be of a desirable minimum width. During the interval between contacting driven guide roll 34 and contacting roll 39 the coated strip does not contact any solid object: in that interval the already preheated coating is brought to fusion temperature and then is solidified, solidification being complete before the coated strip reaches roll 39. Preferably, the procedure is so effected that actual melting of the coating occurs by the time the strip approaches the bottom of chamber 18, thereby making the interval of actual molten condition of the coating an extremely brief one. This is desirable because if the coating is maintained at or above melting temperature too long there is a tendency for the depth of coating to become less uniform than otherwise.

The heating and cooling arrangements of the Figs. 1 to 3 are important, but may be modified somewhat within the scope of this invention. For example, the liquid medium may be omitted partially or entirely. Fig. 4 illustrates a modification where it may be completely eliminated. In describing this form no specific reference will be made to those parts which are duplicates of some of those in Fig. 3.

The major change in Fig. 4 consists in removal of the upper section of the chilling chamber and its squeegee assembly and in withdrawal of the strip directly from the top of the shortened chamber. In doing this, the hood is narrowed to afford a suitable hood 22a having an intake pipe 23a, and a shortened wall structure 14a is substituted for three of the walls 14 of Figs. 1 to 3. The partition 17a and its insulating material 20a 75

are brought downwardly into proximity to the lower guide roll 39, for efficiency in chilling by gas in the chamber 19a. The delivery roll 44 is mounted on the wall structure to receive the strip 5 direct from the roll 39 since the squeegee action is unnecessary where gas is used for the chilling purpose.

The sets of heating elements 48a, disposed in the preheating chamber and controlled by the 10 thermostat 49a, preferably consist of gas jets which burn with reducing flames directed against the strip surfaces. This is true also of the heating elements 50a of the fusion chamber 18 under control of thermostats 52a. If a reducing atmosphere is desirable, and not sufficiently provided by the gas jets, reducing gases may be injected into the heating chambers through the hood pipe 23a. The injected gases may be sufficiently hot for preheating, and hence need to be 20 augmented only by fusing elements in the chamber 18. It is of course to be understood that the temperatures and their relationship to each other and the fusion point of the strip coating must be maintained as previously set forth in the objects and in the description of Figs. 1 to 3.

Although liquid may be used for cooling in conjunction with gaseous heating, the chilling apparatus of Fig. 4 is designed to operate through a gaseous cooling medium, such as cold air, cold 30 neutral gas or cold reducing atmosphere—preferably a cold reducing atmosphere. To this end the pipes 53a receive the cold gas under pressure and discharge it in jet form against the strip. Circulation is maintained by withdrawing the 35 warmer gas through the pipe sections 66a, any suitable pumping and heat-exchanging apparatus being connected to pipes 53a and 66a externally of the chamber in obvious manner.

By filling the chilling chamber with liquid to 40 a level just below the baffle 16, and substituting a pair of squeegee rolls for the delivery roll 44, a liquid cooling medium such as cold oil, or cold water—preferably cold water—may be circulated through the pipes 53a and 66a in lieu of the 45 cold reducing atmosphere.

In Fig. 5 there is illustrated a further modification, having the same three major parts as the preceding forms but having said parts rearranged, and designed to operate with a liquid 50 medium in both heating chambers and a gaseous medium in the chilling chamber. This entire apparatus may be above floor level, or its heating chambers may be disposed in a pit. In view of its close relationship to the previous forms, and 55 its three-step process, a very brief description will suffice.

The heating chambers of Fig. 5 comprise a vertical preheating tank 72, and a fusion tank 73 substantially in the shape of a triangular prism having one side inclined to the horizontal in a direction upwardly and away from the tank 72. An inclined tube 74 which is rectangular in cross section joins the two chambers, both of which are filled with liquid to the indicated level, maintained by the float-switch device 69, 70 in conjunction with any suitable supply means. The tanks have normally closed drain pipes 75, 76.

The upper end of the preheating tank has a slot 77 for the entrance of the strip 7 from the 70 feeding rolls 32b. From these rolls the strip passes downwardly to the guide roll 34b and then is drawn off at an angle through the tube 74, the fusion tank and the baffle 16b by a pair of squeegee rolls 42b, 43b. The latter are located adjacent the strip outlet side of a chilling tank 78,

which at said outlet side has a baffle 79 through which the treated strip is discharged.

The liquid is preheated in the tank 72 by elements 48b that may comprise hot pipes but which preferably consist of electrical units controlled by a thermostat 49b. Likewise the units 50b in the fusion tank may take various forms but preferably comprise electrical elements under control of a thermostat 52b. A vent pipe 80 serves to remove hot vapors and gases adjacent the baffle 16b, thus minimizing the heat transfer between the fusion and chilling chambers.

The strip is quickly chilled in the tank 78 by jets of cold air, cold neutral gas or cold reducing gas, preferably fed against it from pipes 53b. A withdrawal pipe 82 at a higher point in the tank serves to return the warmer gas to the cooling system from which the pipes 53b receive their supply.

If desired, the direction of strip travel in Fig. 5 may be reversed; and the chilling chamber may be removed and the preheating chamber converted into a cooling chamber; this would combine the preheating and fusion units, in effect, into one tank, but such an arrangement is satisfactory in cases where the strip is permitted or caused to travel at slow speed.

While the process and apparatus above described were devised with particular reference to a treatment of strip steel carrying a coating of tin, they may, without the exercise of inventive genius, be employed for a like treatment of other metallic coatings and for combinations in which the base metal is other than steel. Thus, the process and apparatus are operable for like treatment of metallic strip material carrying a coating of copper, or zinc, or nickel, or lead, or bismuth, or other metal which has a melting point lower than the melting point of the base metal, or copper and zinc, or copper and tin, or nickel and copper, or lead and tin, or lead and bismuth, or any other combination of two coating metals the outermost of which shall have a melting point below the melting point of the base metal. Likewise, they are operable for treating metal-coated strips whose base metal is copper, aluminum, nickel, stainless steel, Monel metal or any other metal strip having a higher melting temperature than that of the exposed coating metal.

With reference to the specific combination hereinbefore referred to, of strip steel of relatively low carbon content and of about 30 gauge, carrying on its surfaces electrodeposited coatings of tin, it is noted that the coated strip desirably is preheated to a temperature of about 400° F. in the preheating chamber; that it desirably is further heated to a temperature of about 460° F. in the fusing chamber and is held at the latter temperature for some seconds; and that it is cooled to about 150° F. or below before being contacted by any solid object.

While the invention has been specifically described hereinbefore with particular reference to the treatment of electrically deposited metallic coatings, it is to be appreciated that the process and apparatus of the invention are applicable, without inventive change, to the treatment of coatings which have been applied by the known hot dip method.

Obviously, many other alterations and rearrangements of parts in the several illustrated forms may be made without departing from the spirit and scope of the invention, which may be determined from the appended claims.

I claim:

1. In a method of treating metal strip having a metal plating on surface portions thereof to provide a bright, uniform and adherent coating of improved characteristics, the steps of heating the strip to bring the entire strip to a temperature approaching but short of the melting point of the plating in one heating zone, then further heating the strip in a second heating zone communicating with the first zone to melt the plating, then cooling the strip in a cooling zone communicating with the second heating zone to solidify the plating, controlling the temperatures of the heating and cooling steps so that the plating is melted for only a relatively short period of time, and protecting the strip by non-oxidizing fluids during the heating and cooling steps and the passing between zones.
2. In a method of treating strip steel having a tin surface plating thereon to provide a bright, uniform and adherent coating of improved characteristics, the steps of heating the strip to bring the entire strip to a temperature approaching but short of the melting point of the tin plating in one heating zone, then further heating the strip in a second heating zone communicating with the first zone to melt the tin plating, then cooling the strip in a cooling zone communicating with the second heating zone to solidify the tin plating, controlling the temperatures of the heating and cooling steps so that the tin plating is melted for only a relatively short period of time, and protecting the strip by non-oxidizing fluids during the heating and cooling steps and the passing between zones.
3. In a method of treating metal strip having a tin plating on surface portions thereof to provide a bright, uniform and adherent coating of improved characteristics, the steps of preliminarily subjecting the tin plating and adjacent surface portions of the strip to heat treatment at about 400° F. in a heating zone to bring the entire strip to a temperature approaching but short of the melting point of the tin plating, then subjecting the tin plating and adjacent portions of the strip to heat treatment at a temperature of about 460° F. to melt the tin plating in a second heating zone communicating with said first zone, then cooling the strip at a temperature of about 150° F. to solidify the tin plating in a cooling zone communicating with the second heating zone, controlling the temperatures of the heating and cooling steps so that the tin plating is melted for only a relatively short period of time, and protecting the strip by non-oxidizing fluids during the heating and cooling steps and the passing between zones.
4. In a method of treating metal strip having a metal plating on surface portions thereof to provide a bright, uniform and adherent coating of improved characteristics, the steps of moving the strip in a preliminary heating zone to bring the entire strip to a temperature approaching but short of the melting point of the plating in said zone, then further moving the plated strip downwardly in a vertical path through a second heating zone communicating with the first zone and maintained at a temperature to melt the plating, then further moving said strip downwardly in said vertical path into a cooling zone communicating with the second heating zone and maintained at a temperature to solidify the plating, controlling the temperatures of the heating and cooling steps so that the plating is melted

for only a relatively short period of time, and protecting the strip by non-oxidizing fluids during the heating and cooling steps and the passing between zones.

5. In a method of treating metal strip having a metal plating on surface portions thereof to provide a bright, uniform and adherent coating of improved characteristics, the steps of heating the strip in a segregated heating zone to bring the entire strip to a temperature approaching but short of the melting point of the plating in said zone, then further moving the plated strip downwardly in a vertical path through a second segregated heating zone communicating with the

first zone and maintained at a temperature to melt the plating, then further moving said strip downwardly in a vertical path through a segregated cooling zone communicating with the second heating zone and maintained at a temperature to solidify the plating, controlling the temperatures of the heating and cooling steps so that the plating is melted for only a relatively short period of time, protecting the strip by non-oxidizing fluids during the heating and cooling steps and the passing between zones and restricting substantial circulation between the fluids in adjacent zones.

JOHN S. NACHTMAN.